

July 11, 1933.

H. S. MARSH ET AL

1,917,945

PROCESS OF MAKING FERRIC SULPHATE

Filed Dec. 14, 1928



INVENTORS

Henry S. Marsh  
Carl W. Weesner  
By, S. Tittins, Parmalee & Blenko  
Chairman

## UNITED STATES PATENT OFFICE

HENRY S. MARSH AND CARL W. WEESNER, OF YOUNGSTOWN, OHIO, ASSIGNEES TO SHARON STEEL HOOP COMPANY, OF SHARON, PENNSYLVANIA, A CORPORATION OF PENNSYLVANIA

## PROCESS OF MAKING FERRIC SULPHATE

Application filed December 14, 1928. Serial No. 326,151.

This invention relates to a process of producing ferric sulphate from ferrous sulphate. It relates more particularly to a process of producing ferric sulphate from ferrous sulphate having water of crystallization.

The accompanying drawing is a flow sheet which illustrates the process.

In Patent No. 1,589,610, granted June 22, 1926 to Henry S. Marsh and Ralf S. Cochran for a method of "Reclaiming spent pickling solutions", there is disclosed a method of obtaining copperas crystals from the spent pickling solution. The wet copperas crystals obtained in accordance with the patented process contain seven molecules of water of crystallization. These copperas crystals may be heated to a temperature of 212° F. or higher in order to produce dry copperas crystals having one molecule of water of crystallization.

The present invention has for one of its objects the production of ferric sulphate from dry crystals of ferrous sulphate no matter in what manner the dry ferrous sulphate or copperas crystals are obtained. One method of obtaining dry copperas crystals having seven or less than seven molecules of water of crystallization is by heating the wet copperas crystals obtained by the patented process above referred to.

In accordance with the present invention ferrous sulphate (copperas) crystals containing water of crystallization are heated to a temperature sufficient to drive off all of the water of crystallization and render the crystals substantially anhydrous. This may be accomplished by heating to a temperature of 400-600° F. and preferably by heating to a temperature of about 450° F. This heating, which renders the crystals anhydrous, produces a very friable material which can be easily crushed. The friable material is then finely divided by any grinding means, for example, by crushing it between two steel rollers having smooth surfaces. It is preferable to grind the material to a size such that it will pass through a sieve having 60 meshes to the inch. The ground ferrous sulphate is then heated un-

der oxidizing conditions to a temperature sufficient to convert it into ferric sulphate and ferric oxide. This may be accomplished by heating it in a rotary furnace of the open muffle type to a temperature of 850-925° F., preferably about 900° F. If temperatures higher than these are employed the ferric sulphate tends to decompose, resulting in the formation of an excess quantity of ferric oxide. If lower temperatures are employed some ferrous sulphate will remain unconverted.

The material discharging from the rotary furnace contains about 80% ferric sulphate and about 20% ferric oxide, the ferric oxide having been formed during the heating step in which the material within the kiln had access to the oxygen of the air. The material coming from the kiln is then further treated in order to convert the ferric oxide into ferric sulphate. This may be accomplished by treating the material with a substance containing a sulphate radical. It is preferred to use sulphuric acid for this conversion. The material discharged from the rotary furnace is introduced slowly while stirring into a dilute solution of sulphuric acid. Since during this addition heat is evolved, it is preferred to cool the mixture by any desired means. If the material is added too rapidly to the acid a jellylike mass is formed which is very difficult to control. The addition should, therefore, be made very slowly with constant stirring and cooling of the mixture so that a mushy somewhat liquid and flowable mass is obtained which can be more easily handled and managed than the jellylike mass which would be produced if the addition were carried out in a rapid manner. After the addition of the acid, the material is red in color due to the presence of ferric oxide. This red, mushy mass is heated to a temperature sufficient to convert the ferric oxide to ferric sulphate. The temperatures employed may be from 300 to 850° F., the preferred temperature being about 500° F. This heating accelerates the reaction between the sulphuric acid and ferric oxide, which results in the formation of ferric sulphate. On heating, this change to

ferric sulphate is indicated by the mass changing from a red to a straw or white color. The heating is continued until the mass is thoroughly dry, after which the 5 product is ready for use.

We have described the present preferred manner of carrying out our process. It is to be understood however that the process may be otherwise practiced without departing from the spirit of the invention or the 10 scope of the appended claims.

We claim:

1. In the process of making ferric sulphate, the steps which comprise heating anhydrous ferrous sulphate in the presence of oxygen to about 900° F. to convert it into ferric sulphate and ferric oxide, slowly introducing the mass into sulphuric acid while stirring, and heating the resulting mass to 20 accelerate the reaction.

2. In the process of making ferric sulphate, the steps which comprise heating finely ground anhydrous ferrous sulphate in the presence of oxygen to a temperature of 850-25 925° F. to convert it entirely into ferric sulphate and ferric oxide, and slowly introducing the resultant product into sulphuric acid while stirring, and heating the resulting mass to accelerate the reaction.

30

35

40

45

50

55

60

65

3. The process of making ferric sulphate from ferrous sulphate having water of crystallization, which comprises heating the ferrous sulphate to a temperature of 850-925° F. to convert it entirely into ferric sulphate and ferric oxide, treating the resultant product with sulphuric acid to transform the ferric oxide to ferric sulphate, and heating the resulting mass to about 500° F. to accelerate the reaction. 70 75

4. In the process of making ferric sulphate, the steps which comprise heating finely ground anhydrous ferrous sulphate in the presence of oxygen to a temperature of 850-925° F. to convert it into a mixture containing about 80% ferric sulphate and about 20% ferric oxide, slowly introducing the mixture into a dilute solution of sulphuric acid while stirring and cooling to convert the ferric oxide into ferric sulphate, heating 80 85 the mixture to about 300-850° F. to accelerate the reaction, and thereafter continuing the heating until the mass is substantially dry.

In testimony whereof we have hereunto 90 set our hands.

HENRY S. MARSH.  
CARL W. WEESNER.

95

100

105

110

115

120

125

130